

Aug. 13, 1940.

M. ASIMOW ET AL

2,211,361

APPARATUS FOR CASTING METALLIC INGOTS

Filed Sept. 12, 1939.

FIG. 1.



FIG. 3.



FIG. 4.



FIG. 2.



Inventors:

MORRIS ASIMOW and  
FRANK E. MOONEY.

by: *John E. Jackson*  
their Attorney.

## UNITED STATES PATENT OFFICE

2,211,361

APPARATUS FOR CASTING METALLIC  
INGOTSMorris Asimow and Frank E. Mooney, Gary,  
Ind.

Application September 12, 1939, Serial No. 294,536

1 Claim. (Cl. 22—139)

This invention relates to the casting of metallic ingots, and more particularly to the elimination or material reduction of splashing of the molten metal against the sides of the mold during teeming.

It is well known to those skilled in the art that during the conventional manner of teeming molten metal into ingot molds the splashing of the molten metal against the sides of the mold causes, to some extent, surface defects, such as cracks, seams, etc. This is brought about when the molten metal is first teemed, at which time it impinges on the bottom of the mold or the mold stool (if one is used). The impinging of the molten metal naturally directs the movement thereof onto the relatively cold side walls of the mold, causing particles thereof to adhere, whereupon it is impossible to obtain homogeneity of the surface of the ingot.

It is one of the objects of the present invention to provide an apparatus for casting metallic ingots in such manner that the splashing referred to hereinbefore will be eliminated or materially reduced to such an extent as to minimize the deleterious effects thereof.

Another object is the accomplishment of ends referred to immediately hereinbefore in an inexpensive manner.

The invention, then, comprises the features hereinafter fully described and as particularly pointed out in the claims, the following description and the annexed drawing setting forth in detail the certain illustrative embodiment of the invention, this being indicative of but one of the number of ways in which the principles of the invention may be employed.

In said drawing:

Figure 1 is a sectional elevation of a conventional ingot mold employing the device of the present invention;

Figure 2 is a plan of the mold and device of Figure 1;

Figure 3 is an enlarged plan of the device of the present invention; and

Figure 4 is a side elevation of the showing of Figure 3.

Referring more particularly to the drawing, the numeral 2 designates a conventional "big-end-up" ingot mold of conventional design having the usual necked-in bottom portion 2a, bottom opening 3 and closure or plug 4 by means of which the formed ingot may be stripped from the mold.

As shown more clearly in Figure 2, the ingot mold 2 is shown as having side walls which are corrugated, as indicated at 5, but it will be un-

derstood by those skilled in the art that this is a matter of design which, as such, forms no part of the present invention, and may or may not be employed.

Referring particularly to Figures 3 and 4, the device of the invention comprises a metallic plate, generally designated at 6, which is composed of the same, or substantially the same, composition as the metal of the ingot to be cast. This plate 6 is quite thin, so as to be readily melted by the temperature of the molten metal being teemed, whereby it will become homogeneous therewith.

As shown particularly in Figure 4, the metallic plate 6 is provided with side edges 7 which are directed upwardly in an oblique manner, and the central portion of the plate is provided with a circular aperture, designated at 8.

It is important that the central aperture 8 be larger than the diameter of the pouring stream of the molten metal as it reaches the bottom of the mold 2.

According to a preferred embodiment, the metallic plate 6 is constructed to occupy a position which is 3 per cent to 10 per cent of the total height of the mold above the bottom thereof; but in all events it will occupy a horizontal position in said mold. In addition, the metallic plate 6 is so shaped as to fit in its predetermined position in such manner as to reasonably resist displacement by the molten metal striking it from either above or below.

In the present instance, the plate 6 is shown as having a dimension A of approximately 20 $\frac{1}{4}$  inches and a dimension B of approximately 19 $\frac{3}{4}$  inches in order to fit a square ingot mold matrix having a cross-sectional dimension of 20 $\frac{1}{4}$  inches. In a plate of this size it is preferred to have the radius of the corners of the bottom portion thereof, designated at C, approximately 1 $\frac{1}{4}$  inches and a corner radius D for the upturned portions 7 of approximately 2 $\frac{1}{4}$  inches or to conform to the radius of the mold.

When using a plate 6 of the specific dimensions referred to, we prefer to place the same in the mold 2 at a point approximately 4 inches above its bottom and below the ends of the vertical corrugations 4, if such are employed. When of the dimensions referred to hereinbefore and as so disposed (about 4 inches above the bottom of the mold) we prefer that the central aperture 8 have a diameter E of approximately 14 inches.

When so constructed the metallic plate 6 may be lightly sprung into position against the walls of the mold and is thus enabled to resist the

striking action of the molten metal from either above or below, as previously indicated.

When the diameter E is sufficiently large, it will be obvious that provided, of course, careful teeming practice is observed, the stream of molten metal, after striking the bottom of the mold (or the stool, if such is employed) will be confined entirely to the space below the metallic plate 6 and thus be prevented from impinging upwardly onto the walls of the mold matrix.

When using a mold of the type shown employing the usual "necked-in" bottom portion, designated at 2, the stream of molten metal striking the bottom of the mold will be confined in the rounded end, which will eventually be cut off as scrap. Thus, no splashing will occur which will cause any surface defects on the final product.

While we have shown and described one specific embodiment of the present invention, it will be seen that we do not wish to be limited exactly thereto, since various modifications may be made without departing from the scope of the invention, as defined by the following claim.

5

We claim:

In combination with an ingot mold, a horizontal metallic plate disposed adjacent the bottom of the mold, said metallic plate having an aperture of substantial size to accommodate the teemed stream of molten metal, the side edges of said plate being bent at an angle to enable the plate to snugly grip the mold walls, said plate being composed of a metal which is substantially 10 the same as the metal of the ingot being cast.

MORRIS ASIMOW.  
FRANK E. MOONEY.

15

15